

## UNITED STATES PATENT OFFICE.

RICHARD C. TOLMAN, OF WASHINGTON, DISTRICT OF COLUMBIA.

## MANUFACTURE OF PHOSPHORUS, ETC.

No Drawing.

Application filed January 15, 1921. Serial No. 437,641.

*To all whom it may concern:*

Be it known that I, RICHARD C. TOLMAN, a citizen of the United States, residing at Washington, in the District of Columbia, 5 have invented a new and useful Improvement in the Manufacture of Phosphorus, Etc., of which the following is a specification.

This invention relates to the manufacture 10 of phosphorus and compounds thereof from phosphate rock or other phosphate-containing material and has for its particular objects the economical production of phosphorus or oxygen compounds thereof by a 15 simple and expeditious process which is particularly adapted to large scale operations.

I am aware that in the production of the alloy commercially termed ferro-phos (a description and analysis of ferro-phos can be 20 found in United States Letters Patent No. 1,265,076, page 2, lines 30, 44, 58 and 75) it has been customary to furnace either in an electric furnace or a blast furnace a charge 25 consisting of sand, coke and phosphate rock with which is incorporated a relatively large quantity of iron ore or metallic iron, and the final product produced is the aforesaid ferro-phos for which at the present time there is a relatively limited market. In the 30 production of such a product a not inconsiderable quantity of phosphoric acid may escape in the waste gases, particularly in case an electric furnace is used where the temperatures are so high as to drive phosphorus 35 out of its combination with iron, or in blast furnace operation in cases where the proportion of iron ore added to the burden is reduced below that usual for the production of ferro-phos, and efforts have been made to re- 40 cover this phosphoric acid. It is also known in carrying out such a furnace operation for the production of phosphorus vapors, that the addition of a metal or a metal ore, in particular iron or iron ore, greatly facilitates 45 the process by maintaining a molten bath which serves to keep up the temperature of the refractory slag or in other ways not yet thoroughly understood to facilitate the escape of the phosphorus vapors.

50 My invention is based on the fact that phosphorus compounds of metals, particularly ferro-phos itself, which is a compound or mixture of compounds corresponding to the formula  $Fe_2P$  will, if added to the charge in lieu of iron or other metal or metal ore, serve in an essentially similar manner

to promote the escape of phosphorus vapors, and this product may be recovered and repeatedly used in the production of further quantities of phosphoric acid or phosphorus. 60

In carrying out my improved process I preferably proceed as follows:

A charge consisting of seventy parts phosphate rock, thirty-five parts of sand, ninety parts of coke and about twenty parts by 65 weight of ferro-phos, is introduced into a furnace of any suitable type, for example, a blast furnace or an electric furnace.

In producing phosphoric acid the charge is heated in a blast furnace to a temperature 70 of  $1500^{\circ} C.$  for a period of one hour until substantially all of the available phosphorus has been vaporized and such vapors are conducted to a suitable stove to complete the conversion of the phosphorus into phosphoric anhydride ( $P_2O_5$ ); if desired electrical precipitation of the phosphorus compounds may be resorted to in order more effectively to recover the same. 75

When producing elemental phosphorus the 80 oxidation of the volatilized phosphorus is of course dispensed with and the issuing gases are maintained under reducing conditions.

By my process it is possible to make available substantially the entire phosphorus content of the ore since it is not necessary that a substantial portion of the same shall be converted into ferro-phos as is customary, at the present time, as the ferro-phos agent which I employ in proportions of about 90 10% to 12% for example can be recovered with but a very small amount of loss and utilized in connection with the furnacing of further charges. 85

The ferro-phos is separated and recovered 95 by removing it in a molten form through a suitable tap hole at the bottom of the furnace as is customary in the operation of blast furnaces and electric furnaces.

Having thus described my invention, 100 what I claim and desire to secure by U. S. Letters Patent, is:

1. The process which consists in incorporating in a charge of non-metallic phosphatic material and carbonaceous reducing 105 material a relatively small portion of material consisting of a metallic compound of phosphorus having the catalytic properties of ferro-phos furnacing the charge at a sufficient temperature to effect the volatilization 110 of a quantity of phosphorus corresponding substantially to that represented by the

phosphorus content of the said phosphatic material, recovering the metallic compound of phosphorus from the charge and successively re-utilizing the same for the treatment of further charges of non-metallic phosphatic material and carbonaceous reducing material.

2. The process which consists in incorporating in a charge of phosphate mineral and carbonaceous reducing material a catalytic agent comprising essentially an iron compound of phosphorus having the catalytic properties of ferro-phos, furnacing the charge at a sufficient temperature to effect the volatilization of the greater portion of the phosphorus represented by the phosphorus content of such mineral, recovering the catalytic agent and utilizing the same in a fresh charge of phosphate mineral and carbonaceous reducing material, and repeating such treatment upon such fresh charge.

3. In the process of recovering phosphorus and phosphorus compounds from non-metallic phosphatic material, the step which consists in adding a metallic phosphorus compound having the catalytic properties of ferro-phos to a charge of non-metallic phosphatic material and a carbonaceous reducing material.

30 4. In the process of recovering phospho-

rus and phosphorus compounds from phosphate mineral, the step which consists in furnacing a charge consisting of phosphate rock, carbonaceous reducing material and a relatively small portion of an iron compound of phosphorus having the catalytic properties of ferro-phos to a sufficient temperature to effect volatilization of the phosphorus content of such phosphate mineral.

5. The process of recovering phosphorus and phosphorus compounds from phosphate mineral, the step which consists in reducing phosphate mineral in the presence of carbonaceous reducing material and a catalytic agent consisting essentially of a phosphorus compound of iron having the catalytic properties of ferro-phos, said catalytic agent being present essentially throughout the entire period of treatment.

6. The process of recovering phosphorus and phosphorus compounds from phosphate mineral consisting in reducing phosphate mineral in the presence of a catalytic agent consisting essentially of a phosphorus compound of iron having the catalytic properties of ferro-phos.

Signed at Washington, D. C., this tenth day of May, 1920.

RICHARD C. TOLMAN.